

# UNITED STATES PATENT OFFICE.

MILLS L. CALLENDER, OF NEW YORK, N. Y.

## IMPROVED MATERIAL FOR FILLING SHELLS.

Specification forming part of Letters Patent No. **43,667**, dated August 2, 1864; antedated December 27, 1863.

*To all whom it may concern:*

Be it known that I, MILLS L. CALLENDER, of the State and city of New York, have invented a new and improved material for filling hollow shot, shell, and shrapnel, called "asphalt," "asphaltum," "pitch," "bitumen," or the like substances derived from the distillation of coal, coal-tar, crude coal-oil, certain earth-oils or petroleum, and bitumens. These artificial articles are respectively a residue after distilling off the more volatile products from coal-tar, crude coal-oil, petroleum, earth-oils, and bitumen.

To enable others skilled in the art to manufacture and use my invention, I will proceed to describe its application and operation.

I construct my shot, shell, or shrapnel in any of the known forms, and fill them with the material or materials above specified, either simple or combined with each other, as may be desirable, or combined within organic substances such as niter, sulphur, charcoal, phosphorus, coal-dust, plumbago, lamp-black or graphite, and plaster-of-paris, or the like, to increase its density, hardness and combustibility, and destructive qualities, and also with organic substances such as sawdust, chaff, cotton, tow, tan-bark, or the like, to render the flame more

adhesive and persistent, the proportions of these combinations to be variable, according to the requirements needed. When used to fill shrapnel it serves to fill up the interstices between the balls, holding them firmly to be bored out for the explosive charge, and when shattered by explosion it cleans from the balls and shell easily and cleanly, so the shot or balls will act uniformly. In melting and pouring it does not give off those suffocating fumes so destructive to health that sulphur does, and the shell does not need to be placed in boiling water to insure its filling uniformly, as is the case with sulphur, in this and all cases forming a cheap and useful substitute for sulphur.

What I claim as my invention, and desire to secure by Letters Patent, is—

The use and application of asphalt, asphaltum, or the like, or any of the solid products arising from the distillation of coal, crude coal-oil, coal-tar, rock-oils, or petroleum, natural bitumens, peat, or the like, for filling shell and shrapnel, for the purposes and in the manner as above described.

MILLS L. CALLENDER.

Witnesses:

EDM. F. BROWN,  
Wm. FRANK BROWNE.